

May 13, 1930.

W. M. WEIL

1,758,488

MOLD

Filed Feb. 11, 1929



Fig. 1.



Fig. 2.

INVENTOR  
Walter M. Weil  
BY  
Evans & McCoy  
ATTORNEYS

## UNITED STATES PATENT OFFICE

WALTER M. WEIL, OF CLEVELAND, OHIO, ASSIGNOR TO THE NATIONAL SMELTING COMPANY, OF CLEVELAND, OHIO, A CORPORATION OF OHIO

## MOLD

Application filed February 11, 1929. Serial No. 339,245.

This invention relates to the art of metal founding and more particularly to permanent molds and cores therefor.

This application relates to a specific embodiment of the invention to which broader claims are directed in my copending application filed of even date herewith, Serial No. 339,244, for Frangible molding material.

In the past castings of many metals, ferrous and nonferrous, have been formed in permanent, such as iron, molds in order to produce castings of relatively smooth surface, to obtain an increased rate of production, and to obtain the greatly increased mechanical properties of metals cast in this manner. The above advantages have been particularly noticeable in the case of light aluminum alloys, for example, in the manufacture of automotive pistons. While permanent, such as iron, cores have been employed in permanent mold casting, in many cases it has been found desirable to employ frangible sand cores, partly because of the intricate nature of the interior of the castings. Certain difficulties, however, arise in the use of sand cores in this connection due to the relatively low heat absorbing powers of sand cores. Thus, the exterior of such castings disposed adjacent metal mold parts are chilled relatively rapidly while the interior of such castings disposed adjacent a sand core are cooled relatively more slowly. As a result such castings have been relatively non-uniform in grain structure and physical properties and the physical properties of such castings as a whole have been lessened. The above effects have been particularly noticeable with casting metals of relatively low melting point and relatively high crystallization shrinkage.

An object of my invention is to provide frangible molding material of relatively high heat conductivity. Another object is to provide a frangible core particularly adapted for use in a permanent mold. Other objects are to provide a frangible core for use in the permanent mold casting of metals of relatively high crystallization shrinkage, said core having a relatively high heat conductivity. Another object is to provide a core

comprising a substantial amount of metallic particles.

Other objects will be apparent to those skilled in the art from the disclosures herein made and from the accompanying drawings 55 wherein:

Figure 1 is a vertical section through a permanent mold having associated therewith a core contemplated by my invention, the view of the core being taken on line 1—1 of 60 Fig. 2;

Fig. 2 is an elevation of the core shown in Fig. 1; and

Fig. 3 is a vertical sectional view of a modified form of core, the position of the core being substantially the same as that shown in 65 Fig. 1.

My invention contemplates in one of its forms a frangible core composed of metal particles such as grindings or borings. Such 70 particles may be assembled into a core of the desired shape in a suitable core box by manual manipulation or by the use of mechanical pressure. If desired, a binder may be employed to cause the particles to adhere to each other, such as linseed oil, flour paste, or any suitable commercial core compound, the binder being preferably one which will permit the core to become readily frangible after 75 the casting operation.

In carrying out my invention I may form the core by associating metal particles with sand, the relative proportions of which may be varied to suit the particular conditions in hand. A suitable binder such as described in the preceding paragraph may be employed to cause the core to retain a desired shape. The cores may, of course, be baked, if desired. In forming cores comprising metal particles and sand, the proportion of metal 80 particles may vary within wide limits, for example, from five to ninety-five per cent, depending upon the amount of chilling to be exerted upon the interior of the casting.

In some cases, to prevent adherence of core particles to the casting, or to vary the relative heat conductivity in various portions of the core surface or of the core and outer mold cavity wall, a suitable coating may be disposed upon portions of the core, such coating 95 100

being composed of any suitable material, for example, lime, together with silicate of soda and water.

The composition of the metal particles may vary to a considerable extent. Ordinarily, however, for use with aluminum castings, I find the use of iron, such as cast iron particles, to be very satisfactory, the melting point of the iron being, of course, considerably higher than that of the aluminum casting metal. Other metals may, of course, be employed or, in certain cases, a mixture of metals, for example, for use with aluminum castings the metal core particles may comprise also copper, brass, bronze or aluminum, singly or in mixtures of two or more. Aluminum may in certain cases be employed because of its high heat conductivity and its non-tendency to adhere or weld to other particles of aluminum.

The particular frangibility of core desired may be obtained by varying the nature and size of the metal particles, the amount of sand, the amount and nature of core binder, and the amount of pressure to which the core material is subjected in shaping the core.

In the drawings I have illustrated a permanent mold with which a core according to my invention may be employed. Upon the base 1 are the mold sections 2, which may be suitably disposed in molding position on the mold base by the annular ring member 3 which extends upwardly above the normal upper surface of the base 1. Disposed on the base 1 within the annular ring member 3 is a core 4 formed according to my invention. The core is disposed in the desired position relative to the base 1 and mold sections 2 by disposing the core within the annular ring member 3 and by means of a top portion of the core which extends into the recess 5 in the mold sections. In the present instance the mold and core shown are arranged to form a valve body casting 6 of substantially hollow cylindrical shape having a centrally disposed boss 7 within the casting with struts 8 connecting said boss to the side walls of the casting. The core 4 is shown as provided with the core cavities 9 and 10 to form the boss 7 and struts 8 respectively. The casting metal, such as an aluminum alloy, may be introduced into the mold in any suitable manner, such as for example through the sprue cavity 11 which may be arranged to introduce the casting metal to the top annular portion 12 of the casting 6.

In Fig. 3 I have shown a modified form of core which is additionally hollowed out to provide the cavity 13 in order to lighten the core and to decrease the mass thereof.

By the combination of the permanent mold and my advantageous core it will be noted that the inside and outside of the hollow casting 6 will be cooled at comparable de-

sired rates whereby the casting structure will be relatively uniform and fine-grained within and without, with the well understood advantages. Furthermore, the boss and strut of the casting 6 formed within the core 4 will be cooled at relatively rapid rates, whereby the metal of such boss and struts will be of substantially the same characteristics as the remainder of the casting. By the use of my advantageous frangible core, therefore, a casting having intricate internal surfaces may be readily formed in a permanent mold to provide a casting of uniform strength and structural characteristics.

It will be observed that I have provided frangible molding material of improved characteristics whereby casting metal may be chilled to a predetermined degree to obtain castings of desired physical characteristics.

It will thus be seen that I have provided a core of advantageous characteristics as to heat conductivity whereby aluminum castings of substantially uniform structure and mechanical properties may be formed, and whereby castings may be formed or chilled at the desired rate to impart desired physical characteristics.

It will further be seen that I have provided a frangible core of desirable characteristics which may be readily and economically formed.

It will further be seen that by means of my invention castings having relatively intricate interior surfaces may be readily formed and a desired amount of chilling exerted on their interior.

Furthermore, it is to be understood that the particular forms of apparatus shown and described, and the particular procedure set forth, are presented for purposes of explanation and illustration and that various modifications of said apparatus and procedure can be made without departing from my invention as defined in the appended claims.

What I claim is:

1. In combination, a permanent mold arranged to define the exterior of a casting and to chill relatively rapidly casting metal disposed against said permanent mold, and a frangible core including metal particles arranged to define interior portions of the casting, said core being arranged to chill relatively rapidly interior portions of said casting, whereby the interior and exterior portions of said casting may be of comparatively uniform grain structure and physical properties.

2. In combination, metal mold sections and a frangible core including sand and metal particles, said mold sections and core being arranged to define a casting cavity, whereby casting metal disposed in said casting cavity may be caused to chill relatively uniformly to form chilled castings of improved properties.

3. A permanent mold for casting aluminum alloys and the like comprising, in combination, metal mold sections and a frangible core of sand together with iron particles composed of grindings, borings and the like, said mold sections and core being arranged to define a casting cavity, whereby aluminum alloy castings of uniform physical properties and fine grain structure may be obtained.

10 In testimony whereof I affix my signature.  
WALTER M. WEIL.

15

20

25

30

35

40

45

50

55

60

65